

## UNITED STATES PATENT OFFICE

2,530,804

## LUBRICATING COMPOUND

Sidney Bloomenthal, Chicago, and Fredric E. Wood, McHenry, Ill., assignors to Automatic Electric Laboratories, Inc., Chicago, Ill., a corporation of Delaware

No Drawing. Application October 8, 1948,  
Serial No. 53,594

5 Claims. (Cl. 252—37)

## 1

Our invention relates generally to an improved lubricating compound and more specifically to a lubricant which is especially adapted for use on the bearings of the calling device or "dial" of an automatic telephone.

Telephone dials are subjected to a wide range of temperature in their use in different locations and must not become "sticky" under any conditions. Certain of the gears and bearings in such dials are of brass and others of steel so that lubrication and prevention of corrosion are of prime importance.

The improved compound which we have developed for this purpose consists of 30% of a plastic petroleum such as that sold by the Gulf Oil Company as Plastic Petroleum B, 15% of rust proofing oil such as Ensis No. 211 sold by the Shell Oil Company, and 55% of dibutyl phthalate.

The first component may be of the type described in U. S. Patent No. 2,320,002, granted May 25, 1943 and provides the lubricating qualities at a wide range of temperatures, and remains on the gears and bearings of the device after more volatile components disappear to provide a low coefficient of friction between moving parts even at low temperatures.

The plastic petroleum consists essentially of a mixture of a petroleum lubricating oil with a wax having a wax melting point above about 150° F. and having incorporated therein an amount of aluminum soap such that the ratio of soap to wax is of the order of 1:15.

The second component is a rust preventer and prevents oxygen from attacking the metallic surfaces on which it is present. One such component is described in U. S. Patent No. 2,334,158, granted November 9, 1943.

The rust preventer consists essentially of non-gaseous hydrocarbons containing small amounts of a polycarboxylic acid having at least 16 carbon atoms and of a mutual solvent for hydrocarbons and water, such as an ethylene glycol mono alkyl ether.

The third component is a low volatility solvent for the plastic petroleum and remains liquid by itself to a temperature of —96° F. The presence of this component in the compound aids in the capillary flow of the compound into a bearing when applied to the outside edge thereof. The contact angle on steel for dibutyl phthalate is 0° and for brass is 35°. The compound consequently tends to spread rapidly on steel and stops when it reaches brass. This quality tends to maintain the compound within a bearing when the adjacent parts are of brass.

## 2

While we have described the compound as consisting of certain definite proportions of the various elements, it will be apparent that such proportions may be varied slightly if desired. For instance a slight increase in the amount of dibutyl phthalate reduces the viscosity of the combination and improves the rate of flow during application, while an increase in the amount of the rust inhibitor may give added protection under conditions where severe humidity is encountered.

It will thus be apparent that we have provided a novel lubricating compound which has all the qualities desired for a mechanism which is subjected to wide ranges of temperature and humidity.

## What we claim is:

1. A lubricating compound comprising approximately 30% of a mixture of a petroleum lubricating oil with a wax having a wax melting point above about 150° F. and having incorporated therein an amount of aluminum soap such that the ratio of soap to wax is of the order of 1:15; 15% of a mixture of non-gaseous hydrocarbons containing small amounts of a poly carboxylic acid having at least 16 carbon atoms, and of a mutual solvent for hydrocarbons and water; and 55% of dibutyl phthalate.

2. A lubricant comprising in combination a plastic petroleum consisting of a mixture of a petroleum lubricating oil, a wax having a wax melting point above about 150° F., and an aluminum soap, the soap to wax ratio being of the order of 1:15; a rust preventer consisting of a mixture of non-gaseous hydrocarbons containing small amounts of a poly carboxylic acid having at least 16 carbon atoms and a mutual solvent for hydrocarbons and water; and at least 50% of dibutyl phthalate.

3. A lubricating mixture comprising in combination about 30% of a plastic petroleum consisting of a mixture of a petroleum lubricating oil, a wax having a wax melting point above about 150° F., and an aluminum soap, the soap to wax ratio being of the order of 1:15; at least 50% of a low volatility petroleum solvent; and a rust preventer consisting of a mixture of non-gaseous hydrocarbons containing small amounts of a polycarboxylic acid having at least 16 carbon atoms and a mutual solvent for hydrocarbons and water.

4. A rust proofing lubricant which flows more rapidly on steel than on brass comprising at least 50% of dibutyl phthalate, a small amount of a rust preventer consisting of a mixture of

non-gaseous hydrocarbons containing small amounts of a polycarboxylic acid having at least 16 carbon atoms and a mutual solvent for hydrocarbons and water; and a larger amount of a plastic petroleum consisting of a mixture of a petroleum lubricating oil, a wax having a wax melting point above about 150° F., and an aluminum soap, the soap to wax ratio being of the order of 1:15.

5 A lubricant comprising in combination a non-gaseous hydrocarbon, less than 0.1% of a polycarboxylic acid having at least 16 carbon atoms, a mutual solvent for hydrocarbons and water, a wax having a wax melting point above about 150° F., an aluminum soap, the wax to soap

10 15

ratio being about 15:1, and about 50% dibutyl phthalate.

4 SIDNEY BLOOMENTHAL.  
FREDRIC E. WOOD.

#### REFERENCES CITED

The following references are of record in the file of this patent:

#### UNITED STATES PATENTS

| Number    | Name      | Date           |
|-----------|-----------|----------------|
| 2,396,191 | Morgan    | Mar. 5, 1946   |
| 2,362,767 | Morgan    | Nov. 14, 1944  |
| 2,334,158 | Fuchs     | Nov. 9, 1943   |
| 2,320,002 | Lutz      | May 25, 1943   |
| 2,215,590 | Maverick  | Sept. 24, 1940 |
| 2,104,408 | Wiezevich | Jan. 4, 1938   |